

(No Model.)

J. A. McCLELLAND.

PYROXYLINE FABRIC.

No. 271,493.

Patented Jan. 30, 1883.

Fig. 1.



Fig. 2.



Fig. 3.



Witnesses:

Fred Haynes  
Ed L. Moran

Inventor:

John A. McClelland  
by his Attorney  
Brown & Brown

# UNITED STATES PATENT OFFICE.

JOHN A. McCLELLAND, OF LOUISVILLE, KENTUCKY.

## PYROXYLINE FABRIC.

SPECIFICATION forming part of Letters Patent No. 271,493, dated January 30, 1883.

Application filed October 5, 1882. (No model.)

*To all whom it may concern:*

Be it known that I, JOHN A. McCLELLAND, of the city of Louisville, in the county of Jefferson and State of Kentucky, have invented 5 a new and Improved Pyroxyline Fabric, of which the following is a specification.

The compound produced by treating vegetable fiber with acid, and commonly known as "pyroxyline" compound, is largely used in 10 very thin sheets for various purposes—as, for instance, in the manufacture of collars and cuffs. Where such thin sheets are folded and often unfolded or turned back—as, for example, in the folded parts of collars—the pyroxyline soon breaks in the fold unless re-enforced in some way. To obviate this defect articles have been made with cloth covered with pyroxyline compound; but this is objectionable, 15 because the prepared cloth when doubled or folded is of very considerable thickness.

The object of my invention is to provide a fabric which shall have greater strength, yet be very little, if any, thicker, than sheets of pyroxyline alone, and thinner than sheets of 20 cloth covered with pyroxyline can be made.

To this end my invention consists in a fabric composed of a sheet or sheets of pyroxyline compound, and threads, filaments, or fibers embedded therein, and all extending in 25 one direction. I thus secure a fabric having the necessary strength in one direction in which greater strength may be required, and but little, if any, thicker than the threads, filaments, or fibers used.

In the accompanying drawings, Figure 1 30 represents a piece of my improved fabric. Fig. 2 is a section transverse to the length of the fibers of a small portion of the fabric largely magnified; and Fig. 3 represents a view, similar to Fig. 2, of a piece of a fabric of slightly 35 different formation, but also embodying my invention.

Similar letters of reference designate corresponding parts in all the figures.

A 40 designates a piece of my improved fabric, which is composed of a sheet of pyroxyline compound and threads  $a$ , embedded in the pyroxyline and extending in one direction only in the sheet. These threads may be of very 45 fine cotton twist or cotton yarn, or of any other

vegetable fiber, of animal fiber, such as hair, wool, leather, or intestines, or of other suitable material, and they extend parallel with each other, and may be placed at any desired distance. The fibers are here shown as and 50 may be placed at a distance apart about equal to the diameter of the fibers.

This fabric may be made in any desirable manner. It may be made in large quantities by taking a sufficient number of threads, strands, 55 or yarn or filaments from a beam or spools and conducting them through a reed, whereby they are kept at a proper distance apart, and from which they pass between two pressure-rollers arranged adjacent thereto. The sheets 60 of pyroxyline previously produced are fed between the said rollers, and as they pass with the threads, strands, fibers, or filaments between the rollers the threads, strands, fibers, or filaments are embedded into the sheets of 65 pyroxyline, and are secured to them by the adhesive properties of the compound. By the pressure of the rollers the fibers  $a$  will be forced into one face of the sheet, and on one side will be a very thin covering of pyroxyline 70 over all the threads, while on the other side the pyroxyline will be just flush with the fibers. In the pressing operation the fibers are also flattened, so that they add very little, if any, 75 perceptible thickness to the sheet.

A fabric composed of a single sheet of pyroxyline and fibers or threads is represented greatly magnified in Fig. 3, in which  $b$  designates the pyroxyline in which the fibers are 80 embedded.

Instead of sheets of pyroxyline being fed between the rollers on one side of the fibers, sheets may be fed through on both sides, in which case the fibers  $a$  will be covered equally with pyroxyline  $b$  on both sides of the fabric, 85 as shown magnified in Fig. 3.

This fabric, when composed of fibers embedded between and in two sheets of pyroxyline, is water-proof on both sides, and amply strong without being too thick.

My improved fabric may be used for strengthening the folds in collars made of pyroxyline, for use in the binding of books, pamphlets, &c., for joining the portions of sectional or folding maps or plates in books, for the sweat- 90

bands of hats, and for making or re-enforcing other articles where the material is required to be thin, strong, and water-proof.

What I claim as my invention, and desire to secure by Letters Patent, is—

The fabric composed of a sheet or sheets of pyroxyline compound and threads, filaments,

or fibers embedded therein, and extending all in the same direction, substantially as herein described.

J. A. McCLELLAND.

Witnesses:

CHARLES W. WHITE,  
M. S. THOMPSON.